

June 4, 1935.

H. W. HACKER

2,003,712

PRINTING PLATE BASE

Filed June 21, 1934

3 Sheets-Sheet 1

*Fig. 1.*



*Fig. 2.*



Inventor,  
Horace W. Hacker,

By

Henry T. Bright

Attorneys

June 4, 1935.

H. W. HACKER  
PRINTING PLATE BASE

2,003,712

Filed June 21, 1934 3 Sheets-Sheet 2

*Fig. 3.*



*Fig. 4.*



Inventor,

Horace W. Hacker,

By *Henry T. Bright*  
Attorney

June 4, 1935.

H. W. HACKER

2,003,712

PRINTING PLATE BASE

Filed June 21, 1934

3 Sheets-Sheet 3

*Fig. 5.*



*Fig. 6.*



Inventor,  
Horace W. Hacker,

By *Henry P. Bright*  
Attorney

## UNITED STATES PATENT OFFICE

2,003,712

## PRINTING PLATE BASE

Horace W. Hacker, La Grange, Ill.

Application June 21, 1934, Serial No. 731,737

18 Claims. (Cl. 101—382)

My invention relates to the construction of printing plate bases and also to the construction of lumber from which printing plate bases may be cut to desired sizes. The object of my invention is to so construct lumber of the type specified that the warping, swelling and shrinking thereof when in slab form or cut to sizes for printing plate bases will be reduced to a minimum or entirely eliminated.

- 10 To this end I construct the lumber of a body portion made up of a plurality of small wood blocks each of which blocks, before incorporation in the lumber, has all of its faces provided with a surface seal which will prevent air and moisture from entering the block through any face thereof but which will not destroy the nail penetrable characteristics of the wood block. The blocks thus treated are cemented together preferably with the grain of each block running at an angle 20 with the grain of each block cemented thereto. I then cement to the upper and lower faces of the block assembly thin sheets of wood veneer which will permit the corresponding faces of the plate bases cut from the lumber to be planed to meet dimensional requirements without disturbing the surface seal of any of the small blocks embodied therein. When a printing plate base is cut or sawed from lumber thus formed I again seal the freshly exposed edges of the plate with 30 a suitable metallic tape such as aluminum foil. I have found in practice that the surfaces of the individual blocks can be very effectively sealed by a coating of aluminum paint although other forms of metallic paints or metallic leaf or foil 35 may be employed for the purpose of providing a surface seal for the faces of the blocks embodied in the lumber. My experiments also show that by hermetically sealing all the faces of each of the small wood blocks the assembled material 40 is most effectively protected from atmospheric humidity and its deleterious effect on the stability of such material.

In describing my invention reference will be had to the accompanying drawings wherein

- 45 Figure 1 is a perspective view of a printing plate base cut from lumber with the freshly exposed edges thereof sealed by metallic tape;

Figure 2, a fragmentary perspective view of the base showing the grain relation of adjacent small wood blocks embodied therein and also showing metallic tape partly applied to the freshly exposed edges of the plate;

Figure 3, a view similar to Figure 1, of a modified form of my invention but before metallic tape 50 is applied to the freshly exposed edges of the base;

Figure 4, a view of the modified form similar to Figure 2;

Figure 5, a view similar to Figure 3 of still another modified form of my invention; and

Figure 6, a fragmentary perspective view of the modified form of Figure 5 showing the grain relation of the body portion with respect to the upper and lower surfaces of the base.

Referring to Figures 1 and 2 of the drawings my improved blocking lumber is shown as including a plurality of small wood blocks 10. Before these blocks are assembled in the relation shown I treat all the faces of each block with a surface seal which will not destroy the nail-penetrable characteristics of the wood block, preferably a coating of aluminum paint 11. I then cement the blocks together side to side to form a unitary slab. The upper and lower faces of the resulting slab are then covered by cementing thereto sheets of thin wood veneer 12, such sheets 20 permitting the bases cut from the lumber to be planed to meet dimensional requirements without disturbing the surface seal of the blocks 10. These sheets are so thin that they will not warp the lumber or bases cut therefrom as a result of 25 swelling or shrinking. When a printing plate base is cut or sawed from the lumber thus formed so as to produce freshly exposed faces of the blocks 10 I seal such faces from atmospheric humidity by applying thereto a suitable metallic 30 tape 13, preferably aluminum foil as shown in Figure 2.

In the modified form shown in Figures 3 and 4 the construction is the same as that heretofore described except that I employ two layers of blocks 10a with the abutting surfaces of one layer 35 staggered with respect to the abutting surfaces of the other layer.

While I have shown the body portion of the lumber formed of a plurality of wood blocks, my invention also contemplates the forming of such portion in one piece having all its surfaces hermetically sealed and its upper and lower surfaces respectively covered with thin sheets of wood veneer to permit planing without disturbing any 40 sealed surface of said body portion. When bases are cut from lumber having a one piece surface sealed body portion the freshly exposed edges of the cut base would also be sealed by metallic tape 45 as heretofore referred to.

In the modified form shown in Figures 5 and 6 my improved lumber is also constituted by a body portion formed of a plurality of small wood blocks 14. Before these blocks are assembled in the relation shown all the faces of each block 50 55

are provided with a surface seal such as a coating 15 of aluminum paint. I then cement the blocks together to form a unitary slab. In assembling the blocks 14 of the slab I arrange them 5 so that their cross grain ends will constitute the upper and lower surfaces of the slab. My experiments have shown that wood swells and shrinks in the ratio of about 6 or 5 to 1 as between side grain and end grain. In other words, changes 10 in its dimensions very slightly in the direction of the grain and therefore a distinct advantage is gained by this arrangement with respect to the stability of the height of the lumber or the printing plate base cut therefrom. Also, small blocks 15 cemented together would swell sideways and warp seriously which condition I prevent by the surface sealing of each block heretofore referred to. The upper and lower faces of the resulting slab are covered by cementing thereto thin sheets of wood 20 veneer 16 such sheets permitting the bases cut from the lumber to be planed to meet dimensional requirements without disturbing the surface seal of the blocks 14. Blocking lumber with its upper and lower surfaces formed solely by the cross- 25 grain ends of wood has never been possible before from a practical standpoint, although desirable, because such lumber splits under nailing and renders planing for the purpose of decreasing the height of the lumber or printing plate base cut therefrom exceedingly difficult. By employing 30 the sheets of veneer 16 as shown and described splitting of the lumber or printing bases cut therefrom under nailing is prevented, planing to decrease height becomes an easy operation capable 35 of being accomplished with ordinary wood working tools and the desired practical use of lumber and bases whose upper and lower surfaces are constituted by the cross-grain ends of the wood rendered possible. When a printing plate base 40 is cut or sawed from blocking lumber made in accordance with this modification I also seal the freshly exposed edges of the base with suitable metallic tape such as aluminum foil 17.

By arranging the blocks 14 in pairs and in the 45 row relation heretofore referred to I avoid the use of larger cubical blocks with a corresponding saving in cost and at the same time, this permits the use of smaller blocks which have been found to be more susceptible to perfect sealing.

50 My invention is not limited to the surface sealing of the blocks as in all the constructions shown, with the block surface sealing omitted, the use of sheets of veneer to provide the two major faces of the lumber produces the advantages of preventing splitting of the blocks when penetrated 55 by nails passing through one of the veneer sheets and of enabling printing plate bases cut from the lumber to be more easily planed to decrease height than would be the case where the surfaces 60 of a plurality of blocks constituted the plate receiving face of the base.

When I use the word "veneer" in the claims I 65 mean thin sheets of wood, metal or any other material suitably adapted for the purposes set forth herein.

I claim:

1. Lumber from which printing plate bases are to be cut, said lumber comprising a plurality of wood elements cemented together to form a slab, 70 each of said elements having all its faces hermetically sealed.

2. Lumber from which printing plate bases are to be cut, said lumber comprising a wood body portion having all its surfaces hermetically sealed, 75 and sheets of veneer cemented to and covering

the upper and lower surfaces of said body portion.

3. Lumber from which printing plate bases are to be cut, said lumber comprising a plurality of wood elements cemented together to form a slab, 5 each of said elements having all its faces hermetically sealed before assembly into said slab, and sheets of veneer cemented to and covering the upper and lower surfaces of the slab.

4. Lumber from which printing plate bases are to be cut, said lumber comprising a plurality of wood elements cemented together to form a slab, 10 each of said elements having all its faces hermetically sealed with a metallic coating before assembly into said slab.

5. Lumber from which printing plate bases are to be cut, said lumber comprising a plurality of wood elements cemented together to form a slab, 20 each of said elements having all its faces hermetically sealed with a metallic coating before assembly into said slab, and sheets of veneer cemented to and covering the upper and lower surfaces of the slab.

6. Lumber from which printing plate bases are to be cut, said lumber comprising a plurality of 25 wood elements cemented together to form a slab, each of said elements having all its faces hermetically sealed by a layer of metallic leaf or foil before assembly into said slab.

7. Lumber from which printing plate bases are to be cut, said lumber comprising a plurality of 30 wood elements cemented together to form a slab, each of said elements having all its faces hermetically sealed by a layer of metallic leaf or foil 35 before assembly into said slab, and sheets of veneer cemented to and covering the upper and lower surfaces of the slab.

8. The method of producing a printing plate base which consists in hermetically sealing all the 40 faces of each of a plurality of wood elements, cementing said elements together to form a slab, cutting the base to desired size from the slab thus formed, and then hermetically sealing the edges 45 of the base which were freshly exposed by the cutting operation.

9. The method of producing a printing plate base which consists in hermetically sealing all the 50 faces of each of a plurality of wood elements, cementing said elements together to form a slab, cutting the base to desired size from the slab thus 55 formed, and then hermetically sealing the edges of the base which were freshly exposed by the cutting operation by covering said edges with metallic tape.

10. Lumber from which printing plate bases are 60 to be cut, said lumber comprising a plurality of wood elements cemented together in superimposed layers to form a slab, and with the abutting faces of the elements in one layer staggered with respect to the abutting faces of the elements 65 in adjacent layers.

11. Lumber from which printing plate bases are to be cut, said lumber comprising a plurality of 70 wood elements cemented together in superimposed layers to form a slab, and with the abutting faces of the elements in one layer staggered with respect to the abutting faces of the elements in adjacent layers, and sheets of veneer cemented to and covering the upper and lower surfaces of the slab.

12. Lumber from which printing plate bases are to be cut, said lumber comprising a plurality of 75 wood elements cemented together to form a slab with the cross grain ends of the elements constituting the upper and lower surfaces of the slab 80

respectively, and sheets of veneer cemented to and covering said surfaces.

13. Lumber from which printing plate bases are to be cut, said lumber comprising a plurality of 5 wood elements cemented together to form a slab with the cross grain ends of the elements constituting the upper and lower surfaces of the slab respectively, each of said elements having all its faces sealed before assembly into said slab, and 10 sheets of veneer cemented to and covering said upper and lower surfaces of the slab.

14. Lumber from which printing plate bases are to be cut, said lumber comprising a plurality of 15 wood elements cemented together to form a slab with the cross grain ends of the elements constituting the upper and lower surfaces of the slab, each of said elements having all its faces sealed with a metallic coating before assembly into said slab, and sheets of veneer cemented to and covering 20 said surfaces.

15. The method of producing a printing plate base which consists in sealing all the faces of each of a plurality of wood elements, cementing said elements together to form a slab with the cross 25 grain ends of the elements constituting the upper and lower surfaces thereof, cementing to and

covering said surfaces with veneer sheets, cutting the base to desired size from the material thus formed, and then sealing the faces of the wood elements which were freshly exposed by the cutting operation.

16. Lumber from which printing plate bases are to be cut, said lumber comprising a wood body portion having all its surfaces hermetically sealed and its upper and lower surfaces constituted by 10 the cross grain of the wood, and sheets of veneer cemented to and covering the upper and lower surfaces of said body portion.

17. Lumber from which printing plate bases are to be cut, said lumber comprising a plurality of 15 wood elements cemented together to form a slab, and sheets of veneer cemented to and covering the upper and lower surfaces of the elements respectively.

18. Lumber from which printing plate bases are to be cut comprising sheets of veneer constituting 20 the top and bottom of the lumber and at least one layer of wood blocks held between the sheets each of said blocks having all its surface hermetically sealed.

HORACE W. HACKER. 25